

Jan. 31, 1933.

J. H. SWAN, 3D

1,895,527

PAPER MANUFACTURE

Filed Aug. 30, 1929



Inventor

Joseph H. Swan III

Maréchal and Moé

Attorneys

## UNITED STATES PATENT OFFICE

JOSEPH H. SWAN, 3d, OF MIDDLETOWN, OHIO, ASSIGNOR TO THE GARDNER-RICHARDSON COMPANY, OF MIDDLETOWN, OHIO, A CORPORATION OF OHIO

## PAPER MANUFACTURE

Application filed August 30, 1929. Serial No. 389,421.

This invention relates to the manufacture of paper, and particularly to the manufacture of board adapted for use in the making of containers and the like.

5 One of the principal objects of the invention is to provide a paper or board which is grease proof and moisture proof, is sufficiently flexible and elastic to permit bending, is substantially odorless and tasteless, stands up 10 well in use and does not objectionably deteriorate on standing for considerable intervals of time, and is commercially economical.

Another object of the invention is to provide a superior grease proofing and moisture 15 proofing coating for paper or board of this character.

Other objects and advantages of the invention will be apparent from the following description, the accompanying drawing and 20 appended claims.

In the drawing, which discloses a preferred embodiment of the invention

Fig. 1 is a side elevational diagrammatic view of apparatus which is constructed to 25 apply the coating to form the paper product of this invention; and

Fig. 2 is a vertical sectional view on an enlarged scale of a piece of container board made in accordance with this invention.

30 This invention is particularly applicable to the rendering of paper or board, such as container board, impervious to grease, so that containers made therefrom may be used for packaging greasy or oily substances

35 which would otherwise penetrate through the package. When such a product is used for packaging foodstuffs, such for example as peanut butter or the like, it is particularly desirable that the surface of the container

40 board be substantially tasteless and odorless. The coating should be of such character as to form an impervious layer on the board without pin holes which destroy the effectiveness of the coating, and it should be sufficiently flexible and elastic to permit the bending of the board, such as is necessary in the formation of the box or container, without cracking.

45 The coating should also be of a durable nature, and one that will stand up 50 well in use and will not objectionably de-

teriorate upon standing for considerable intervals of time. In accordance with the present invention, a coating composition is provided which has superior qualities, and a coated paper product is formed which is unusually efficacious in satisfying the above requirements. 55

Referring to the drawing, the paper or board to be coated is carried by a reel 10 supported in suitable bearings on a frame 60 11 mounted on the foundation. The paper or board indicated at 12 passes over a guide roll 13 and thence between the nip of driven rolls 14 and 15 which form a coating press. Each of the rolls 14 and 15 is mounted in slidably 65 bearings 16 provided with suitable adjustment screws 17 passing through a collar 18 carried by the frame 11, an adjustment nut 19 and a lock nut 20 serving to permit desired horizontal adjustment of the bearings. This 70 permits the rolls 14 and 15 to be adjusted relatively to each other to bring the rolls into contact with the desired operating pressure, forming a trough indicated at 21 above the nip which is closed at each end by a suitable 75 deckle member 22. Coating solution of a grease proofing nature is supplied to the trough 21 by pipe 23 having a control valve 24. The paper 12 passing through the trough and between the nip of the rolls receives a 80 coating on one side thereof, the thickness of the coating being regulated by the pressure at the nip.

The grease proofing coating composition applied at this point comprises glycerine, a 85 water solution of sodium silicate, and an alkali metal compound adapted to maintain the coating in an alkaline condition to prevent deterioration of the coating film. The addition of glycerine to the sodium silicate 90 imparts characteristics of flexibility and resiliency to the coating and tends to prevent cracking thereof when the board is bent in the formation of the container, and also improves the spreading and the grease proofing 95 qualities of the coating with the production of a substantially impervious film or layer. Other polyhydric alcohols, for example glycols such as ethylene glycol, can be used with satisfactory results in substantially the same 100

manner as glycerine. Other alkali metal silicates, such as potassium silicate, can be used in place of sodium silicate, but from the standpoint of economy the latter is preferred. 5 The presence of an alkali in the coating prevents deterioration of the same upon standing, and serves to increase the effective life of the coating. Various alkali metal compounds such as sodium carbonate, ammonia, 10 sodium hydroxide, borax and the like may be used for this purpose. Alkaline compound of sodium or potassium are preferred to ammonia, inasmuch as the latter is subject to evaporation while the former retain the coating permanently in the desired stable condition.

In the preparation of the coating composition, the alkali metal silicate is first made up in a relatively concentrated water solution. 20 Thus where sodium silicate is used, a solution containing in excess of about 15% sodium silicate is preferred. Satisfactory results may be secured with solutions containing from about 15% to 60% sodium silicate by 25 weight. The alkali metal compound is also made up in water solution, or may be dissolved directly in the sodium silicate solution. These ingredients are then mixed with the glycerine. Satisfactory results have been 30 secured with compositions containing from 15% to 40% by volume of glycerine, and 60% to 85% by volume of a water solution of sodium silicate of the above proportions, this composition containing about 1 to 2% by 35 weight of an alkali metal compound adapted to preserve the alkalinity of the coating.

As an example of a very satisfactory coating composition, the following is mentioned: 40 Sodium silicate solution of about 38% strength and glycerine are mixed in the proportions of about 25% by volume of glycerine and 75% by volume of the sodium silicate solution. To this composition is added about 1% to 2% by weight of sodium carbonate. 45 The board 12 with the coating on the upper surface thereof then passes across a plurality of rotatable drying drums 28 mounted in bearings 29 carried by a frame 30, the under surface of the board contacting with the upper portions of the drying drums. These 50 may be the conventional steam heated drying cylinders, and are maintained at the usual temperatures which is customary in the drying of paper. The board then passes around 55 a strain roll 31 so that the coated surface is then underneath, and returns with the upper uncoated surface in contact with a portion of the bottom of the surfaces of the drying drums 28. As many drying drums may be 60 provided as is necessary to secure the proper drying of the coating.

A board which is given only a grease proofing coating is subject to deterioration when exposed to the atmosphere, and particularly 65 when exposed to water or dampness. In ac-

cordance with the present invention, an overlying water insoluble wax coat is applied over the grease proof coating. Very satisfactory results are secured with paraffin, beeswax, montan wax, or other well known water insoluble waxes. From the standpoint of economy and ease of application paraffin is preferred for this purpose. This combination of an oil insoluble coat with a water insoluble overcoat applied as herein described 70 gives advantageous results. The overlying wax coat not only protects the under grease proofing coat from exposure and deterioration, but also adds to the water proofness and 75 moisture proofness of the coating, which is particularly advantageous in the packaging of deliquescent substances such as crackers, for example. The wax coat also renders the 80 surface of the board in contact with the materials or foodstuffs to be packaged tasteless and odorless.

For the purpose of applying the top wax coat, a press comprising a lower roll 35 and an upper contacting roll 36 with which the under coated surface of the web 12 contacts, 85 is provided. The lower roll 35 dips within a trough 37 containing a bath of paraffin 38 maintained in molten condition by a suitable steam coil 39. Rotation of roll 35 within the 90 bath of molten paraffin provides a surface film upon this roll which is transferred to the contacting roll 36 and thence to the paper web in the form of a thin film over the base coating. The coated web then passes over a suitable 95 guide roll 40, or additional drying means 100 as desired, and thence is wound on a reel 41.

In order to further improve the quality of the paper product, the paper or board is first subjected to a sizing treatment before the 105 coating is applied. Thus the board, or the layer of the board forming the outer surface which receives the coating is preferably a "hard sized" sheet, or one which has been made up from paper stock to which a sufficient quantity of size, such as rosin size or 110 paraffin size, has been added as to materially retard the rate at which water or ink penetrates into the sheet. Very satisfactory 115 results are secured by forming a sheet from paper stock to which rosin size has been added in the beater in the proportion of about 80 pounds of size to 1200 pounds of pulp. A sheet which will stand up for approximately five minutes or over in the water drop test, 120 which means that water will not penetrate the sheet in that time, is satisfactory. Or the sheet may be given a surface sizing by an application of a size to the surface of the formed web, using suitable conventional sizing materials such as above specified. The grease 125 proofing coating is then applied to the hard sized sheet, or on top of the surface sizing, the grease proof coating being thereby prevented from objectionably sinking into the sheet 130 with resultant deterioration.

Referring to Fig. 2, a section through a preferred sheet of board is disclosed, which is found to be highly effective for use in containers for the packaging of greasy materials, 5 and which protects the materials from water and damp atmospheric conditions. This sheet comprises inner layers of ordinary board stock 45, with an intermediate layer 46 of asphaltic material, such as an emulsion of 10 asphalt and clay. The outer surfaces of the board are formed of good grade liner stock, providing a bottom liner 47 and a top liner 48. The top liner 48, which is adapted to 15 form the interior of the container and to receive the grease proof coating, is a hard sized sheet.

This board as above described may be formed on a conventional cylinder mold machine having a number of molds to form the 20 various layers or plies of the sheet, these plies being brought together and united in the ordinary manner. Thus a conveying felt of the forming machine passes first across a cylinder mold containing the bottom liner stock 25 and forms a web, and then passes successively across cylinder molds provided with board stock, asphalt emulsion, board stock, and finally top liner stock to form the complete built-up sheet of container board. The 30 top liner may be surface sized instead of having the size distributed throughout the sheet.

After formation, the board is then passed through the coating machine as above described, and a layer of grease proofing composition 49 of the character specified above is applied to the surface of the hard sized liner, and a final top coat of a water insoluble wax 50 is applied over the grease proofing coat. This sheet is thus protected from 40 water and moisture tending to penetrate from the outside into the interior of the container by the intermediate asphaltic layer, and is made effectively grease proof, water proof and moisture proof by the coating applied to 45 the interior surface of the container.

While the form of invention disclosed herein constitutes a preferred embodiment thereof, it is to be understood that the invention is not limited to this precise form, and that 50 changes may be made therein without departing from the scope of the invention which is defined in the appended claims.

What is claimed is:

1. A paper product of the character described comprising a hard sized sheet having a coating including a polyhydric alcohol, an alkali metal silicate and an alkali metal compound which is alkaline in character, the 55 coating being primarily maintained on the surface of the sheet by the sizing in the sheet.

2. A paper product of the character described comprising a surface sized sheet having superposed upon the surface sizing 60

coating including a polyhydric alcohol and an alkali metal silicate.

3. A paper product of the character described comprising a hard sized sheet having a flexible surface coating of a grease proofing 70 composition which is primarily maintained on the surface of the sheet by the sizing in the sheet, and a water insoluble wax layer overlying the grease proofing coating.

4. A paper product of the character described comprising a surface sized sheet having superposed upon the surface sizing a grease proofing composition, and a top layer 75 of a water insoluble wax overlying the grease proofing composition. 80

5. A paper product of the character described comprising a sheet having a grease proofing coating of an alkaline composition of a polyhydric alcohol, an alkali metal silicate and an alkali metal compound which is 85 strongly alkaline in character.

6. A paper product of the character described comprising a sheet having a grease proofing coating including essentially a polyhydric alcohol and oil insoluble adhesive, the 90 polyhydric alcohol being present in an amount in excess of 25% by weight on the weight of the oil insoluble adhesive to impart substantial flexibility to the coating.

7. A paper product of the character described comprising a sheet having a grease proofing coating including an alkaline mixture of glycerine and sodium silicate, applied from a solution containing from 60% to 85% by volume of a water solution of sodium silicate containing from 15% to 60% by weight of sodium silicate, and from 15% to 40% by volume of glycerine, and solution also containing a small amount of an alkali metal compound which is alkaline in character. 95 100 105

8. A paper product of the character described comprising a container board made up of a plurality of plies of paper with an intermediate asphalt layer, the surface of said board having a grease proofing coating and an overlying coat of a water insoluble wax. 110

9. A paper product of the character described comprising a container board made up of a plurality of plies of paper with an intermediate asphalt layer, the surface of said container board which is adapted to form the interior of a container having a grease proofing coating including a polyhydric alcohol and an alkali metal silicate, and a coat 115 of a water insoluble wax overlying the grease proofing coating. 120

10. A paper product of the character described comprising a container board made up of a plurality of plies of paper with an intermediate asphalt layer, the top liner of said container board which is adapted to form the interior of a container being hard sized and having a grease proofing coating on the surface of said hard sized liner and a coat 125 130

of a water insoluble wax overlying the grease proofing coating.

11. A container board adapted for the packaging of greasy materials, comprising a 5 laminated sheet made up of a plurality of plies of paper with an intermediate water proofing and moisture proofing layer, one surface of said laminated sheet having a substantially odorless and tasteless non-fibrous 70 grease proofing coating applied thereto and maintained primarily on the surface of the said sheet.
12. A container board adapted for the packaging of greasy materials, comprising a 15 laminated sheet made up of a plurality of plies of paper with an intermediate water proofing and moisture proofing layer, the outer ply of said laminated sheet on the side which is adapted to form the interior of a 20 container being a sized paper having on the exposed surface thereof an overlying grease proofing coating.

13. A container board adapted for the packaging of greasy materials, comprising a 25 laminated sheet made up of a plurality of plies of paper with an intermediate water proofing and moisture proofing layer, one surface of said laminated sheet having a 90 grease proofing coating and an overlying 30 coat of a water insoluble wax.

14. A container board adapted for the packaging of greasy materials, comprising a 35 laminated sheet made up of a plurality of plies of paper with an intermediate asphalt layer, the surface of said laminated sheet which is adapted to form the interior of a 105 container having a non-fibrous grease proofing coating applied thereto and maintained primarily on the surface of the said sheet.

15. A board product of the character described comprising a laminated board made up of a plurality of plies of paper with an intermediate water proofing and moisture proofing layer, one surface of said laminated 110 board having a grease proofing coating including an oil insoluble adhesive and a polyhydric alcohol.

16. A board product of the character described comprising a laminated board made 50 up of a plurality of plies of paper with an intermediate asphalt layer, one surface of said laminated board having a multiple layer 115 grease proofing and moisture proofing coating applied thereto.

17. A board product of the character described comprising a laminated board made up of a plurality of plies of paper with an intermediate water proofing and moisture proofing layer, one surface of said laminated 120 board having a multiple layer grease proofing and moisture proofing coating applied thereto.

18. A paper product of the character described, comprising a hard sized sheet having 125 85 a flexible surface coating of a grease proofing

composition including an oil insoluble adhesive which covers the exposed surface of the sheet, and which is primarily maintained on the surface of the sheet by the sizing in the sheet to provide a durable grease proofing 70 coating.

19. A paper product of the character described, comprising a surface sized sheet having superposed upon the surface sizing a 75 flexible coating of a grease proofing composition including an oil insoluble adhesive which covers the surface sizing, and which is primarily maintained on the surface of the sheet by the sizing to provide a durable grease proofing coating.

In testimony whereof I hereto affix my signature.

JOSEPH H. SWAN, III.

85

90

95

105

110

115

120

125

130